

# UNITED STATES PATENT OFFICE.

THOMAS JEFFERSON HADLEY, OF WINNIPEG, MANITOBA, CANADA.

## ELECTRICAL INSULATING COMPOUND.

1,103,285.

Specification of Letters Patent.

Patented July 14, 1914.

No Drawing.

Application filed September 29, 1913. Serial No. 792,497.

*To all whom it may concern:*

Be it known that I, THOMAS JEFFERSON HADLEY, of the city of Winnipeg, in the Province of Manitoba, Canada, have invented certain new and useful Improvements 5 in an Electrical Insulating Compound, of which the following is the specification.

The invention relates to an improved compound especially designed for use in connection with electrical installation and the object of the invention is to provide a compound which can be readily applied to an electrical conductor and will effectively insulate said conductor from the adjoining 10 structure, a particular feature of the invention being that the compound is inexpensive and durable and readily compounded.

The composition consists of the following ingredients combined in the following proportions: Coal tar, 8 gallons; kerosene, 2 15 gallons; Portland cement, 2 gallons; Japan drier, 1 gallon. The coal tar, kerosene and Portland cement are first placed in a vessel and thoroughly mixed. The Japan drier 20 is then added. The amount of Japan drier 25 may vary depending whether one requires

a heavy viscous mixture or a more mobile mixture.

This composition when applied on an electrical conductor will effectively insulate it. 30 The resultant mass is pliable and very slightly sticky, and will retain its original properties for an indefinite period. The cement gives it body and binds the compound while the oil appears to form a solvent which permits of a close mixture of the cement and tar. 35

What I claim as my invention is:

1. An electrical insulating compound consisting of coal tar eight gallons, kerosene oil 40 two gallons, Portland cement two gallons and Japan drier one gallon.

2. An electrical insulating compound comprising coal tar 8 gallons, kerosene oil two 45 gallons, Portland cement two gallons and Japan drier.

Signed at Winnipeg this 27th day of June 1913.

THOMAS JEFFERSON HADLEY.

In the presence of—

G. S. ROXBURGH,  
R. FOSTER.